

May 10, 1932.

A. E. MILLINGTON

**1,857,316**

## MANUFACTURE OF WALL BOARD AND THE LIKE

Filed May 26, 1927

11 Sheets-Sheet 1



Fig. 1,

Inventor

Arthur E. Millington

By his Attorneys

Cooper, Kerr & Danham

May 10, 1932.

A. E. MILLINGTON

1,857,316

MANUFACTURE OF WALL BOARD AND THE LIKE

Filed May 26, 1927.

11 Sheets-Sheet 2



Inventor  
Arthur E. Millington  
By his Attorneys  
Cooper, Kerr & Dunham

May 10, 1932.

A. E. MILLINGTON

1,857,316

MANUFACTURE OF WALL BOARD AND THE LIKE

Filed May 26, 1927

11 Sheets-Sheet 3



May 10, 1932.

A. E. MILLINGTON

1,857,316

MANUFACTURE OF WALL BOARD AND THE LIKE

Filed May 26, 1927 11 Sheets-Sheet 4



Fig. 4,

*Arthur E. Millington*  
Inventor  
By his Attorneys  
*Cooper, Kerr & Dunham*

May 10, 1932.

A. E. MILLINGTON

1,857,316

MANUFACTURE OF WALL BOARD AND THE LIKE

Filed May 26, 1927

11 Sheets-Sheet 5



May 10, 1932.

A. E. MILLINGTON

1,857,316

MANUFACTURE OF WALL BOARD AND THE LIKE

Filed May 26, 1927

11 Sheets-Sheet 6



May 10, 1932.

A. E. MILLINGTON

1,857,316

MANUFACTURE OF WALL BOARD AND THE LIKE.

Filed May 26, 1927

11 Sheets-Sheet 7



Arthur E. Millington  
By his Attorneys  
Cooper, Kerr & Dunham

May 10, 1932.

A. E. MILLINGTON

1,857,316

MANUFACTURE OF WALL BOARD AND THE LIKE

Filed May 26, 1927

11 Sheets-Sheet 8



Fig. 13



May 10, 1932.

A. E. MILLINGTON

1,857,316

MANUFACTURE OF WALL BOARD AND THE LIKE

Filed May 26, 1927

11 Sheets-Sheet 9



Fig. 15,



Fig. 17,



Fig. 16



Fig. 18,

Inventor

Arthur E. Millington

By his Attorneys

Cooper, Kerr & Dunham

May 10, 1932.

A. E. MILLINGTON

1,857,316

MANUFACTURE OF WALL BOARD AND THE LIKE

Filed May 26, 1927

11 Sheets-Sheet 10



May 10, 1932.

A. E. MILLINGTON

1,857,316

MANUFACTURE OF WALL BOARD AND THE LIKE

Filed May 26, 1927

11 Sheets-Sheet 11



## UNITED STATES PATENT OFFICE

ARTHUR E. MILLINGTON, OF SAN FRANCISCO, CALIFORNIA, ASSIGNEE, BY DIRECT AND MESNE ASSIGNMENTS, TO THE UNITED STATES NATIONAL BANK OF PORTLAND, OREGON, AS TRUSTEE

## MANUFACTURE OF WALL-BOARD AND THE LIKE

Application filed May 26, 1927. Serial No. 184,288.

This invention relates generally to the manufacture of wall, insulating, and sound-deadening boards and similar materials, and has particular reference to a new material 5 of the kind mentioned; and to mechanism for producing such material.

A broad object of the invention is to make the waste from sawmill and lumbering operations economically useful, thereby providing a way of supplementing the rapidly 10 diminishing available lumber supply.

Another object of the invention is to provide a method of producing fibrous material suitable for use in making wall boards and 15 the like which will yield fibre which is chemically unweakened and which will lend itself to interlacing or mutual entanglement in the board-making operations. An incidental object is to provide a method which can be carried on at a very low expense and with a 20 minimum outlay for manufacturing equipment.

Another object of the invention is to provide a wall board which will have great 25 strength and a very high degree of insulating quality. This is accomplished partly by the peculiar nature and relation of the fibres giving the strength characteristic and which provides innumerable air gaps or spaces; and 30 partly by the fact that the non-fibrous parts of the bark from lumbering operations is included in the board, such non-fibrous material possessing to a high degree the desirable insulating qualities.

Another object is to provide a novel combination of mechanisms, and interconnections 35 between them, which are adapted to carry out the novel method and produce the novel product at a relatively high production rate and at a minimum cost.

Other objects and advantages will be apparent from the description hereinafter given and from an examination of the drawings, which accompany and form a part of this 40 specification.

In said drawings:

Fig. 1 is a plan view showing in somewhat diagrammatic form the relation of chipping, screening, and digesting sections of the apparatus.

Fig. 2 is a continuation of Fig. 1, and shows the stock tanks for the cooked material and some of the devices subsequently called into action.

Figs. 3 and 4 are views from different angles of the chipper and some of the mechanism associated therewith.

Figs. 5 and 6 are respectively side and end views of the chip screening apparatus.

Figs. 7 and 8 are respectively a front elevation of the digester and the gearing used for driving the digester.

Figs. 9, 10 and 11 show details of the devices for distributing the cooked material among the storage tanks.

Fig. 12 is a section on the line 12—12 of Fig. 2 and shows among other things the fibre separator machines.

Fig. 13 is a top plan view of the mechanism shown in Fig. 12.

Figs. 14, 15, 16, 17 and 18 collectively show the construction of the fibre separating machines.

Figs. 19 and 20 are complemental sheets showing the board-forming apparatus as viewed from 19—19 and 20—20 of Fig. 2.

Fig. 21 is a plan view of a flow box.

Stated in a general way, the present invention includes what may be termed a softening process of preparing the material for subsequent operations, such preparation consisting mainly in cooking sawmill waste of all kinds, including the natural percentage of bark, in a weak solution of soda ash. Preferably, this cooking operation is carried on in a rotary digester and in the presence of live steam, although the cooking may be effected in other ways. The term digester is used herein as a matter of convenience. As will be apparent later on, the device designated by that name does not, as a matter of fact effect digestion of its contents within the usual meaning of the term.

In actual practice the rotary digester is filled approximately to half of its capacity with wood waste which has been reduced to suitable sizes, or under a maximum size, and the digester then filled with water within per cent, approximately, of its capacity. At any time before the cooking operation is

started, commercial soda ash may be added to the contents of the digester in any suitable way, although all that is necessary is to dump in the proper amount of the soda ash for 5 the amount of material in the digester, thereby making unnecessary, chemical houses, solution vats, and the like. The most desirable results are obtained by using about one and one-half pounds of soda ash for each cubic 10 foot of the material to be treated, although the amount of soda ash may be varied for different woods. The digester is then closed by a manhole cover, and rotation of the digester started to tumble the contents. The 15 digester may be run for a short period to cause a thorough commingling of its contents, after which steam may be turned on, or the starting of the digester and the admission of the steam may be simultaneous. 20 The rotation of the digester and the admission of the steam is continued until substantially all of the gums, resins, and the like holding the fibres together are separated and largely removed from the fibres. While this 25 is going on, a bleeder is operating, preferably in an automatic manner, to remove some of the liquor from the condenser so as to maintain the desired temperature and compensate for or offset the effects of steam condensation. 30

The preferred amount of soda ash per cubic foot of material, that is, one and one-half pounds per cubic foot, will give a solution in the digester of about  $3\frac{1}{2}$ ° Baumé. 35 Owing to the steam condensation and operation of the bleeder carrying off the liquor, the Baumé will, however, gradually be lowered until at the end of the cooking operation the Baumé will be 1° or possibly less. 40 Even if the nature of the material requires a greater amount of soda ash, the Baumé will seldom exceed 6° with a decrease in the Baumé as the cooking proceeds.

The operation, as so far described, takes 45 from twelve to twenty-eight hours, according to the volume of the digester contents and temperature of the steam employed. Relatively high steam temperatures may be used, because of the fact that the digester contains 50 a great deal more water than is customary in similar processes, the great volume of water preventing the scorching or charring of the material, which has in the past been one obstacle in the way of shortening the 55 cooking by increase of temperature. The steam is preferably admitted near the center of the rotary digester, or on a central line, so that it aids or supplements the rotary movement of the digester in effecting a thorough tumbling and cooking of the contents 60 of the digester.

When the cooking operation is completed the chips and pieces of bark will still have substantially their original sizes and shapes. 65 In other words, they are not disintegrated or

dissolved by the cooking treatment, this being one important distinction between the present process and prior processes for making pulp to be used in the manufacture of paper and similar materials. The fibres in the woody matter also will be in chemically unweakened condition, thereby differing in another respect from the prior processes. 70

A satisfactory form of digester or cooker for the purpose is illustrated in the drawings, 75 Fig. 7. This part of the apparatus consists of an unlined globular shell 20 rotating on a horizontal axis and provided with a manhole and cover of the usual type. This manhole is, in the filling position of the digester, 80 at the top, and the water, soda ash, and raw material are dumped or poured in and the manhole cover bolted in position. The steam is admitted through a pipe 21 extending through the center of one of the supporting 85 trunnions for the digester a bleeder 22 extending outward from the trunnion at the opposite side. The admission of steam is controlled by the usual valve 23, and the bleeder is equipped with the usual automatic 90 trap 24. Associated with the bleeder is a hand operated valve 25 and pipe so placed and constructed that it may be operated, when the cooking operation is completed, to relieve the digester from the larger part of 95 its internal pressure and much of the liquid contents.

Diametrically opposite the manhole on the digester is a blow-off pipe and valve 27 which is adapted to be connected by a suitable union 100 28 to a pipe or hose 29 leading to a sewer. The interior of the digester around the outlet to the blow-off pipe is provided with a perforated plate or screen 26 of sufficient fineness to retain in the digester substantially all 105 of the useful material while allowing the liquor to pass without much interference. This construction is much cheaper and simpler than the usual blow-pit used in pulp-making operations, and results in a corresponding reduction in the cost of plant construction. 110

After the liquor has drained off, the remaining contents may be washed by means of a hose or the like inserted through the manhole, until all of the liquor and its contents are washed out, such washing also removing substantially all of the remaining dissolved and soluble matter not carried off with the liquor. This washing operation in the digester consumes only a few minutes, and may under certain conditions be omitted in view of a subsequent washing operation later mentioned which is effected after the material leaves the digester. 115

After the liquor has been withdrawn and the washing in the digester, if any, completed, the blow-off pipe union 28 is disconnected from the drain and the digester given a half turn to permit the cooked and washed ma- 120

terial to drop from the digester into a receptacle 31. This receptacle, as shown in Fig. 7, is preferably constructed with its sides converging toward the bottom to concentrate the material toward a screw conveyor 32. This screw conveyor carries the cooked and washed material from the receptacle 31 to a chain conveyor 33, Figs. 2, 9 and 10, comprising cross-bars 34 of the usual type and inclined as shown in Fig. 10. The run of this conveyor which is used for conveying the material passes above and in close contact with a screen 35. This screen has small perforations or is of comparatively fine mesh. Located above the screen and cross bars 34 is a set of shower pipes 36 which thoroughly spray and wash the material as it is carried up over the screen 35, the water passing through the screen to a sewer conduit. When the washed material finally leaves the end 37 of the screen it is carried by the conveyor 33 over an imperforate surface 39 and above a series of tanks 42, 43 and 44. The imperforate surface referred to is provided with openings 45, 46, 47, above the tanks 42, 43, 44, respectively. Each of the openings is equipped with a sliding gate. When the conveyor mechanism is running as previously described, the gate for the opening 45 is open about one-third of the way; the gate for the opening 46, two-thirds of the way; and the gate for the opening 47 is fully opened so as to clear the entire opening. In this way the material carried by the conveyor is distributed equally among the three tanks, this distribution being maintained until the three tanks are filled to the desired extent. The tanks are collectively of sufficient capacity to receive a number of batches of cooked and washed material coming from the digester, and when filled in the way described serve as a means for averaging the results from the various cookings, thereby insuring a substantial uniformity of the contents, regardless of slight variations in the cooking process. A duplicate set of tanks and associated features may be placed at the other side of the conveyor 33.

The tanks 42, 43 and 44 are equipped with rotary agitators 48, driven by any suitable connections, as by the gearing and shafts shown, and which are connected to a motor, or other suitable source of power. Each of the tanks 42, 43, 44 is connected to a water supply. Preferably the water used in the tanks is condensation water from the board drier forming a part of a complete plant, and the best results are obtained if this water is warm enough to give a temperature of approximately 100° F. in the tanks.

While in storage in the tanks 42, 43, 44, the material is maintained in about a 5 per cent suspension, but before removing it for the next operation, sufficient water is added to reduce the proportion to about 2 per cent material and 98 per cent water. This add-

ed water is mainly for convenience in pumping and conveying the material to the point where the next operations are performed.

Associated with the three tanks is a centrifugal stock pump 51, connected to a header 52, the header in turn being connected by valve-controlled pipes 53 to the different tanks, so that the pump may conveniently be connected to any tank desired.

The pump is also connected by a suitable pipe 55 to an elevated flow box 56, Figs. 12 and 13, containing three compartments 57, 58, 59, Fig. 21. The material first enters the compartment 57 and passes through a regulating gate 61 into the compartment 58 and through an outlet 62 to the upper one of a series of fibre separators described in detail later on. The compartment 59 is to receive overflow from compartment 57, over a dam or weir 63, the compartment 59 being provided at its bottom with an outlet 64 for returning the overflow and stock carried therein to the storage tank from which it came. The return connections for the overflow are not shown in detail, but any construction satisfactory for the purpose may be used.

The stock leaving through the outlet 62 enters a spread box 66 serving to spread the flow to form a flat sheet conforming in width to the throat or intake opening 67 of a fibre separator 68, constituting the first or upper one of a series of similar machines. The flow through the spread box 66 is controlled and regulated by a suitable adjustment of the sliding gate 61. The embodiment illustrated in the drawings employs four of the separators arranged on a descending incline. They are all alike, with a single difference herein-after explained, and a description of one of them, accompanied by an explanation of the difference mentioned, will be sufficient.

The separator 68 resembles in a great many respects the swing hammer machines used for pulverizing ores and clays, and, to a limited extent, certain vegetable growths, such as kelp and sugar cane. The machines which have been used for pulverizing purposes are, however, unsuitable for the present purpose, and certain changes have been made to secure the desired effect upon the material passing through the machine.

The prior machines employed various forms of gratings and cutting bars, giving a cutting and pulverizing action which is highly undesirable in the present treatment of the raw stock.

The machine 68 employed in the present instance comprises a rotor 71, Figs. 14 and 15, consisting of a number of disks supporting cross bars or rods 72, upon which rods are loosely pivoted iron plates or centrifugal hammers 73. The throat or intake opening 67 of the machine 68 opens into a hopper provided with bars 74 which are adjustable to cooperate with the ends of the plates 73.

when the rotor is turning in the direction of the arrow. The best results, for present purposes, are obtained when the bars 74 are so adjusted as to leave an appreciable gap 5 between the ends of the plates and the bars.

In the prior machines used for the other purposes above mentioned, the plates 73 usually were constructed from stock  $\frac{1}{8}$  of an inch thick, but in the present machine these plates 10 are  $\frac{1}{16}$  of an inch thick, and approximately twice as many of the lighter and thinner plates are used as were used in the older construction, the lighter and thinner plates being held apart on their pivots by spacers 15 between them.

In the prior machines the lower part of the enclosure for the rotor was composed of a series of sharp-edge cutter bars cooperating with the pivoted plates or hammers 73 to cut 20 the material between the hammers and the bars. As a result, the previous machines pulverized the material, an effect which is undesirable for present purposes. The present machines have a bottom plate 75 with a 25 smooth concave surface substantially concentric to the axis 76 of the rotor 71. The plate 75 in the separator is provided with numerous circular perforations, Fig. 17, which are preferably  $\frac{1}{4}$  of an inch in diameter, although the size of the perforations may be 30 slightly increased or decreased according to the result desired.

Considered as a whole, the increased number of light-weight plates or hammers 73, 35 and the smooth interior and perforations described, cooperate to brush the material against the interior of the machine, thereby causing a separation of the fibres, as distinguished from a cutting or pulverizing action upon them, the hammers finally brushing the fibres through the perforations. The second of the separators 78 is the same, in 40 every respect, as the machine 68 just described in detail. The separators 81 and 82, however, are different from separator 68 in 45 one respect, as in both separators 81 and 82 the bottom plate 75, instead of having circular perforations, is provided with a series of slots 83 (Fig. 18) which are preferably 50  $\frac{1}{16}$  of an inch wide and 1 inch long, the slots 55 extending in a circumferential direction or parallel to the direction of movement of the plates 73. This slotted construction results in retaining all of the material in the interior of the separator until the fibres have been separated sufficiently for them to brush through or escape through the slots.

By the time the material has passed 60 through the last separator, the woody portions will have been reduced to fibres having a hair-like appearance, many of the fibres being of considerable length and substantially free one from another. Others of the fibres will be only partially separated one 65 from another, resulting in what is, in effect,

a coarse fibre. Such coarse fibres are not removed by any screening process, as they are highly desirable in the present process and product.

For the average wood waste, the four fibre 70 separators operate consecutively upon the material, and means are provided for directing the flow from one to the next until the separating operation is completed. This directing means is, however, so constructed that 75 by opening a suitable by-pass, one or more of the machines may be cut out.

In addition to the by-pass mechanism, means are also provided for regulating the water content of the flow, a change in the 80 water content effecting a change in the results produced in each machine. In other words, the progress of the material through any one of the separators may be sped up or retarded by regulating the amount of water, a decrease in the amount of water causing a longer dwell and greater degree of fibre separation, and an increase in the supply resulting in a lesser degree of separation and a coarser condition of the fibre. This by-pass 85 and water control apparatus, and the consequent difference in the condition of the fibres, as will be clearer later on, combine to afford a means of controlling the density, hardness, and sound-deadening qualities of the final 90 products. It also gives a flexibility in the operation of the separators which makes it possible to adjust or regulate their operation according to the species of the wood in 95 the raw material.

When the material has passed through the perforated plate 75 in the fibre separator 68, it drops upon a slide or trough 91, Fig. 14, which conducts it to the receiving opening of the separator 78, which opening is like the opening 67 previously described in connection with the refiner 68. The separator 78 is provided with a similar slide or trough 92 leading to the separator 81, and the separator 81 in turn has a trough or slide 93 leading to the final separator 82. Located near the lower end of each of the slides or troughs 91, 92, 93 is a dam 95 which may be lowered to prevent the flow from the preceding separator entering the next one. When the dam is lowered, a removable plug, not shown, is withdrawn from an outlet 96, allowing the flow which would otherwise have passed to the next separator to fall upon a chute or trough 97, which, at its lower end, communicates with a spout 98, inclined as shown, and provided with openings in its bottom above the stock tanks. These openings may be equipped with suitable gates or slides so as to direct the flow of the stock to any tank desired.

While the slides 91, 92 and 93 were previously described in such a way as to indicate that they are continuous surfaces, it is preferred to construct them of wire mesh which will allow a separation of the water and stock. 130

Below the screens 91, 92, 93 are imperforate slides or bottoms, provided with outlets 101, 102, 103, each equipped with a valve 104. Normally the valves are closed, and after the spaces under the screens have filled up with water, the further flow is directed into the separators. Whenever it is desired to remove a part of the water before the flow enters the next separator, the valve in the corresponding outlet 101, 102, or 103, is set to allow all or any desired part of the water content to escape into a trough 105 leading to the return water tank 106. In addition to the outlets 101, 102, 103, for allowing part of the water to escape, a separate water supply pipe 107, Fig. 14, of any suitable construction is provided with a valve 108 whereby water may be added at the throat of each separator, with a consequent speeding of the action in that particular machine. Only one of the pipes 107 is shown in the drawings, but it will be readily understood that each separator has the same water supply arrangement for the purpose stated.

The flow of material leaving the final separator, or the last one in operation if one or more of the separators has been cut out, goes to the trough 98, which has previously been referred to in connection with the water control, and then to whichever one of a series of stock tanks 111, Figs. 2 and 12, is in condition to receive the stock. These stock tanks are equipped with rotary agitators 110, each driven by a gear connection 112 and 113 through a shaft 114 connected in any desired way with a motor 115. The stock is suspended in the tanks in a volume of water sufficient to give it about a 2 per cent consistency.

The stock tanks 111 may, if desired, be employed for waterproofing the stock. A suitable waterproofing material is the ordinary paper-makers' sizing, consisting of rosin in semi-liquid or liquid form, the amount of rosin employed being substantially one-half of one per cent of the dry weight of the material. This rosin is first introduced into the tanks, and the agitation of the contents of the tanks continued until the fibres are thoroughly coated. An amount of alum about equal to the amount of rosin, is then introduced into the tanks, causing a precipitation and fixing of the rosin on the fibres.

The tanks 111 are all connected to a header 118 equipped with a separate valve 119, whereby the tanks may be independently connected to and disconnected from the header. The header is connected to a stock pump of suitable construction and capacity for carrying the stock to the starting end of the board-forming machine shown in Figs. 2, 19 and 20.

The board-forming machine used is fully described in an application filed by Arthur E. Millington on the 26 day of May, 1927, Serial No. 194,289, and needs not, therefore, be described in detail in the present application.

It is sufficient for present purposes to say that the board-forming machine comprises a coarse-mesh Fourdrinier wire 121, Figs. 19 and 20, inclined upwardly from the breast roll 122 or starting end, with suitable guides 123 and deckles 124 to permit forming and maintaining a pool 125 of considerable depth at the foot of the incline and extending for a distance of ten or twelve feet lengthwise of the wire.

The wire is, as stated in the application referred to, run at a low speed as compared with the usual Fourdrinier wire, the speed preferably being approximately from twenty to thirty linear feet per minute. As also explained in the application referred to, this results in the fibres tending to move endwise with the flow of water through the meshes of the Fourdrinier wire, thus causing a considerable percentage of the fibres to be at right angles or other angles to the face of the finished board. In the finished board the fibres will, therefore, be entangled or interlaced, thereby contributing in a marked degree to making the finished board wholly self-sustaining, that is, capable of resisting breaking and other strains without the use of binders or fillers of any kind to cause mutual adhesion of the fibres.

The apparatus and process as so far described can be used in producing the fibrous stock and the finished board from any of the softer woods. It is, however, preferable to use what may be termed the long-fibre woods, particularly satisfactory results having been obtained from the waste derived from sugar and white pines, and from fir. Fir is particularly suitable for the purpose, and a percentage of fir included in the waste from other woods increases the desirable qualities of the finished product.

As stated at the outset, the raw material includes the natural percentage of bark. Bark contains some fibrous material and a large percentage of non-fibrous material. The non-fibrous material is particularly valuable in wall-board and similar products because of its high insulating qualities, approaching cork in that respect. The apparatus and method as a whole is adapted to retain the larger part of the non-fibrous part of the bark in the stock, and after the refining operation the fibrous part of the stock engages or enmeshes the non-fibrous pieces. This relation of the fibres and non-fibrous material is thereafter maintained and is found in the finished board.

It will be noted that the apparatus as so far described makes no provision for screening out coarser fibres, provided that the fibres are under a useful maximum. In actual practice the stock comprises fibres of widely varying sizes and lengths, the long fibres giving the resistance to breaking strains and the shorter fibres serving as binders to tie the longer

fibres together. The short fibres incidentally insure the proper enmeshment of the non-fibrous portions of the bark. These various sizes and lengths of the fibres and the portions of the bark all contribute to the production of a board which contains the air voids and cells which have been found so desirable in insulating and sound-deadening material.

The waste from the sawmill and lumbering operations, including slabs, edgings, limbs, and the like, may be reduced to pieces of a suitable size for the subsequent operations in any suitable way. Preferably, however, a conveyor system, designated generally as 131, Figs. 1, 3 and 4, conveys the waste above the hopper 132 of a chipper 133. This chipper is preferably of the disk type, with knives 134 which are adjustable to regulate the size of the chips. The process as a whole is facilitated by keeping all of the waste under a maximum thickness of one inch and a length of approximately two inches. The length is not of importance, but the maximum length indicated is preferred, because it has been found to be the best one for satisfactory cooking and fiberizing.

After passing through the chipper the chips fall into a bin 140, preferably having sides and bottoms directing the chips to a belt-conveyor 141. The conveyor is inclined upward to elevate the chips to a hopper or chute 142 leading into the interior of a rotary chip screen 144, Figs. 1 and 5. This screen consists of two tubular screens 145 and 146, one within the other, the inner screen being of any predetermined mesh which will screen out from the chipped waste any part of the material which is too coarse or too long for efficient use. The outer screen 145 is of a finer mesh than the inner screen and is intended principally to screen out dust and particles which are too small to serve a useful purpose in the final product.

The screen, as shown, is on an inclined axis, and when the screened material eventually reaches the lower end the rejects leave the inner screen and may be carried by a suitable conveyor (not shown) to a re-chipper or crusher or disposed of in any desired way. The material leaving the lower end of the outer screen drops upon a belt-conveyor 148 which runs to a chip-bin above the digester hereinbefore described, from which bin the chipped material is removed for use in charging the digester.

In describing the various features of the mechanism and the various steps involved in the process, it has been necessary to state the operations in considerable detail, and it is thought therefore that the summary of operation usual at this point may be omitted.

While the description has gone into great detail with respect to the various features and ideas, it is not the invention to be limited to

such details except as they may be included in the following claims.

What is claimed is:—

1. The process of making wall board from saw mill waste and the like which includes the steps of reducing the waste to pieces which will pass through a screen of a predetermined mesh, boiling the reduced waste in a weak solution of soda ash long enough to separate the gums and resins from the fibers and loosen the fibers to soften the waste, washing the material to remove the gums and resins from the fibers, and then mechanically effecting separation of the fibers whereby to provide a finished board of soft, self-sustaining material capable of resisting breaking and other strains without use of a binder or filler. 70 75 80

2. The process of making wall board from saw mill waste and the like which includes the steps of reducing the larger pieces of waste to pieces which will pass through a screen of a predetermined mesh, agitating the waste in a weak solution of soda ash in the presence of live steam long enough to 85 90 95 separate the gums and resins from the fibers in the waste, said solution not being in excess of two pounds of soda ash for each cubic foot of the material to be treated, washing the material to remove the separated gums and resins from the fibers and then subjecting the washed material to frictional action whereby to effect separation of the fibers in the material whereby to provide a finished board of soft self-sustaining material capable of resisting breaking and other strains without use of a binder or filler. 100

3. The herein described process of making wall board which comprises running saw mill waste including bark through a chipper, screening out all material over certain dimensions and subjecting the remainder to steam under pressure and a solution of soda ash to soften the material, said solution not being in excess of two pounds of soda ash for each cubic foot of the material to be treated, and then subjecting the material to frictional impacts to effect separation of the fibers therein, then suspending the material in a large volume of water and agitating same to cause further separation of the fibers and a thorough commingling of the fibrous and non-fibrous portions of the material, and then employing said water as a vehicle for carrying the suspended material to the starting end of a board making apparatus. 110 115 120

4. A process of making wall board which comprises reducing the waste from a lumbering operation to pieces under a predetermined maximum thickness and length, tumbling such reduced material in the presence of live steam and a solution of soda ash to effect softening of all of the material and a partial liberation of the fibers in the woody portions of the material while maintaining 125 130

substantially unchanged the size of the pieces, and then mechanically separating the liberated fibers, mixing the fibrous and non-fibrous material with a great volume of water and agitating the mixture to effect further separation of the fibers and a commingling of the fibrous and non-fibrous material, and then delivering the water with the commingled materials in suspension therein to

5 a board forming apparatus whereby to provide a finished board of soft self-sustaining material capable of resisting breaking and other strains without use of a binder or filler.

5. The herein described process of making wall board which comprises reducing saw mill waste, including bark, to pieces which are all under a predetermined thickness and length, tumbling said reduced waste in the presence of live steam under pressure and a

10 solution of soda ash under Baumé 5 to effect softening of the fibers in the waste and to dissolve the gums and resins binding the fibers together, washing the material to remove dissolved and water soluble matter

15 from the material, subjecting the washed material to a brushing action to effect separation of the fibers, agitating the separated fibers in a large volume of water to effect commingling of the fibers, suspending the

20 fibers in a water proofing solution, and conducting said solution and suspended material to the starting end of a board making apparatus whereby to provide a finished board of soft self-sustaining material capable of

25 resisting breaking other strains without use of a binder or filler.

6. A process of making insulating wall board which comprises reducing the waste, including bark, from a lumbering operation

30 to pieces under a predetermined maximum thickness and length, subjecting such reduced material to agitation in the presence of steam pressure and a weak solution of soda ash to effect softening of all of the material and

35 a partial liberation of the fibers of the woody pieces of the material, said solution not being in excess of two pounds of soda ash for each cubic foot of the material to be treated, washing such softened material in such a way as

40 to remove the soda ash and any dissolved and water soluble matter while retaining the solids and fibrous material, mechanically separating the fibers in the woody pieces of the

45 washed material, agitating the fibrous and

50 non-fibrous material in water to effect commingling of said materials, and then forming the commingled material into boards and drying same whereby to provide a finished board of soft self-sustaining material ca-

55 pable of resisting breaking other strains without use of binders or fillers.

60 7. A process of making wall board which comprises reducing the waste, including bark, from a lumbering operation to pieces

65 under a predetermined maximum size, sub-

jecting said reduced material to agitation in the presence of steam and a weak solution of soda ash of sufficient volume to protect the material from charring and effect softening of all of the material, said solution not being in excess of two pounds of soda ash for each cubic foot of the material to be treated, washing such softened material in such a way as to remove dissolved, detached and soluble matter while retaining the solids and fibrous material, subjecting the washed material to the successive action of fiber separators arranged in series to effect separation of the fibers in the woody part of the waste, suspending the separated fibers in water and removing the water as an incident to forming the fibers into boards.

70 8. A process of making wall board which comprises reducing the waste, including the bark, from a lumbering and saw mill operation to pieces under a predetermined maximum size, subjecting such reduced material to agitation in the presence of and by steam and a solution of soda ash of less than Baumé 6 total to soften the material and remove the resins and gums therefrom without substantial disintegration of the material, removing the solution and resins and gums contained therein, washing the material to remove any remaining soda ash, gums and resins while retaining the solids and fibrous material, mechanically separating the fibers in the woody parts of the washed material, then alining and interlacing the fibrous material and enmeshing the solids and forming same

75 into a sheet and then pressing and drying same whereby to provide a finished board of

80 soft self-sustaining material capable of resisting breaking and other strains without use of binders or fillers.

85 9. A self-sustaining wall board made from saw mill waste and the like, composed of a porous mass comprising entangled wood fibers from which the natural gums and resins have been dissolved in such a way as to leave the fibers unweakened by chemical treatment, and some of which have been wholly separated and others partially separated by mechanical treatment whereby to produce a

90 wall board capable of resisting breaking and

95 other strains without use of a binder.

100 In testimony whereof I hereto affix my signature.

ARTHUR E. MILLINGTON.

120

125

130